

Sept. 14, 1943.

P. E. QUENEAU ET AL

2,329,483

BEARING

Original Filed May 27, 1938

Fig. 1.



Fig. 2.



Fig. 3.



Fig. 4.



INVENTORS  
PAUL ETIENNE QUENEAU  
BY WILLIAM ALVIN MUDGE  
G. P. Weller  
ATTORNEY.

Patented Sept. 14, 1943

2,329,483

# UNITED STATES PATENT OFFICE

2,329,483

## BEARING

Paul Etienne Queneau, Copper Cliff, Ontario, Canada, and William Alvin Mudge, New York, N. Y., assignors to The International Nickel Company, Inc., New York, N. Y., a corporation of Delaware

Original application May 27, 1938, Serial No. 210,370. Divided and this application February 5, 1941, Serial No. 377,428

13 Claims. (Cl. 308—237)

The present invention relates to anti-friction and anti-galling metals and alloys and, more particularly, to composite anti-friction and anti-galling bearings characterized by high strength and resistance to corrosion.

It is well known that there have been many bearing (anti-friction) alloys containing principally lead, tin, antimony, copper, etc., but these have only a moderate resistance to certain types of corrosion and were generally soft. Usually these alloys possessed low melting points and low resistance to high temperature. Other bearing metals, such as bronze, lead-copper, or hard lead type have fulfilled some of the requirements of hardness and strength, but do not satisfy the most exacting corrosion-resisting requirements, particularly of sea water corrosion. Furthermore, good and adequate lubrication is necessary at all times. Case hardened steels have relatively good anti-galling properties and very high strength and hardness, but have little or no resistance to corrosion. A malleable, high strength metal or alloy having good resistance to corrosion in most media and good anti-galling or anti-friction properties when used for rolling and/or sliding friction has not been commercially available. The art has been confronted with a problem requiring the production or treatment of alloys having relatively high tensile strength, such as about 100 or 140 to 160,000 pounds per square inch tensile strength with a minimum of 20 per cent elongation, having excellent corrosion resistance to salt water and certain other agents operating without galling under sliding and rolling friction, and being self-lubricating. In connection with the use of alloys of the aluminum-copper-nickel series described in the U. S. Patent No. 1,572,744 to Merica and the U. S. Patents Nos. 1,755,554, 1,755,555, 1,755,556 and 1,755,557 to Mudge, under conditions where anti-galling is required, it has been customary in the past to treat the surface by "wiping" a very thin layer of tin or solder thereon. This was satisfactory in service only as long as the tin remained intact. However, since the tin or the anti-friction ("layer") metal was only in mechanical contact with the underlying ("base") metal, the former soon wore off and failed to provide the necessary protection against galling. Moreover, the bearing surface possessed poor resistance to sea water corrosion.

Although many attempts have been made to solve the outstanding and vexatious problem confronting the art, none, as far as is known, has been wholly successful and satisfactory when carried into practice on an industrial scale for the production of commercial products.

We have discovered that the aforesaid problem may be solved in a remarkably simple manner and that the art may be provided with an

improved anti-friction and anti-galling structure having high strength and corrosion resistance.

It is an object of the present invention to provide a new anti-friction and anti-galling bearing alloy characterized by good resistance to corrosion and the ability to operate under conditions of sliding and/or rubbing friction without failure through galling or seizing.

10 It is another object of the present invention to provide an improved composite anti-friction and anti-galling structure of high strength and good resistance to corrosion.

15 Other objects and advantages will become apparent from the following description taken in conjunction with the accompanying drawing, in which:

20 Figs. 1 and 2 are views representing photomicrographs of the present improved anti-friction and anti-galling structure illustrating desirable types of bearing surfaces;

25 Fig. 3 represents a photomicrograph of a cross section of an improved anti-friction and anti-galling structure showing "mountains" or projections on the roughened face of the underlying base or foundation stratum peeping through the applied layer of anti-friction metal; and

30 Fig. 4 is similar to Fig. 3 and illustrates schematically a cross section of an embodiment of the invention employing a plurality of layers of metal, the first or intermediate layer acting as a bonding layer.

35 Broadly stated the bearing contemplated by the present invention comprises a layer of anti-friction metal or alloy applied to the bearing face of a metal base to form a composite material. Adequate and effective anchorage for the coating is obtained by roughening the bearing face of the base to provide hills or projections separated by valleys or depressions. In the finished bearing the bearing surface comprises tops of the hills as islands of harder material surrounded by the layer of softer anti-friction metal in the 40 valleys or depressions. The layer metal and the base metal are preferably diffused into each other by heat treatment. As a result, a novel and efficient bond is produced between the layer and the base materials and the bearing combines the 45 hardness and resistance to corrosion of the base metal with the anti-galling properties of the layer metal. Furthermore, the bonding provides a means of keeping this layer intact with the base so that it will not strip or wear off in the 50 service as usually occurred heretofore in the cases of the conventional wiped tin layer.

55 Processes of roughening the base, of applying the coating to the base, of heat treating the coated base, and of machining the composite bearing are disclosed in our copending application, Serial No. 210,370, filed May 27, 1938, now

Patent No. 2,241,789, granted May 13, 1941, of which the present application is a division.

It is to be observed that the nature of the bond between the base and layer metals or alloys will vary with the chemical and physical properties of these materials. Some will bond more readily than others, some produce a greater thickness in the bonding than others, and in some cases the amount of bonding is very small. Nevertheless, the superior performance of and new results produced by the novel heat-treated products is direct evidence that the heat treatment is beneficial and desirable. It is also true that the heat-treatment produces a certain amount of sintering and intra-diffusion in the layer metal, when applied by spraying, for example, and that this is of distinct advantage in reducing (but not completely eliminating) the porosity thereof. Similarly, the heat-treatment would eliminate or would tend to eliminate a considerable percentage of occluded gases such as would be present in layer metal applied by electrodeposition, and, even in sprayed layers would assist in eliminating or reducing brittleness. In the broadest sense, therefore, the heat-treatment serves the multiple purpose of bonding the layer material to the base material in varying degrees, of sintering the particles of the layer material together, and of eliminating undesirable occluded gases, thereby ameliorating the physical properties thereof. In corrosion-resisting services this latter feature is of great importance. When the heat-treatment is conducted in an atmosphere of reducing gases, it tends to eliminate oxides by reduction, particularly in the cases of sprayed coatings.

It is to be noted that the porous nature of sprayed metal coatings is distinctly advantageous with regard to their use as bearing surfaces. This porosity enables them to absorb a considerable amount of lubricating medium and hold the latter in reserve for periods in which, for one reason or another, the lubrication is not adequate. For example, the bearing on which a sprayed coating has been applied may be subjected to a vacuum to remove the air from the pores and then immediately immersed in a liquid lubricant under high pressure to impregnate the bearing with the lubricant.

As those skilled in the art will readily understand, the selection of the exact nature or properties of the layer material must be governed by the type of service desired. For example, if the corrosive medium in which the alloy must work is a sulphuric acid medium, a lead-containing layer alloy would preferably be chosen; if the corrosive medium is sea water, a silver-cadmium layer alloy containing about 10 to 95% of silver with the balance cadmium would preferably be chosen. Particularly satisfactory results have been obtained within the range of about 65 to 95% silver, and a preferred range is about 75% to 85% silver, with the balance substantially cadmium. A similar choice may also be made with reference to the base metal. For example, if high tensile strength is desired combined with lightness (low specific gravity) one or more of the aluminum alloys of the age-hardening type would be selected; if high strength and hardness with corrosion resistance are desired, one of the alloys of the aluminum-copper-nickel type previously mentioned would preferably be chosen.

The present invention contemplates the use of a layer alloy which improves the corrosion resistance as well as the anti-galling properties of

the base alloy, such as a silver-cadmium coating on steel. For special purposes, a generally considered base metal may also be used as a layer metal in order to impart specially desired properties together with bearing characteristics, such as, for example, the use of bronze on nickel alloys or the use of aluminum alloys on steel.

From a broad point of view, when resistance to corrosion is involved, the selection of the layer material is based in part upon the position of the materials involved in the well established electromotive series. For best results, not only the chemical properties of the layer material must be considered but also its position in the electromotive series. Its position in the series should, in general, be lower than that of the base material, i. e., the layer material should be cathodic with respect to the base material. A selection on the foregoing basis will serve to decrease the likelihood of corrosion of the layer material.

For the purpose of securing best results, especially in connection with sea water, we prefer to use a base constituted of nickel base alloys. Typical of such alloys are nickel-copper alloys sold under the trade-mark "Monel" and nickel-chromium-iron alloys sold under the trade-mark "Inconel." We may also use iron base alloys, such as the carbon and alloy steels, or copper base alloys, such as brasses, bronzes and nickel silvers, or aluminum base alloys, preferably of the age-hardening type, such as duralumin.

For the layer, we prefer to use silver or cadmium or alloys thereof. We may likewise employ anti-friction materials, such as tin, zinc, aluminum, lead, copper, antimony, carbon (graphite), indium, beryllium, bismuth, gold, palladium, platinum, silicon, rhodium, etc., singly or in combination. Indium is of particular benefit in increasing the corrosion resistance of certain of the cadmium and copper base alloys.

When it is difficult or impossible to obtain a diffusion bond between the layer and the base metals, an intermediate layer of a satisfactory bonding element or alloy will first be coated on the base metal prior to application of the selected layer material. In this manner, an anti-friction and anti-galling structure or bearing is produced comprising a base, an intermediate layer, and a bearing layer. Upon subsequent appropriate heat-treatment, the desired bond would be obtained, thus producing a structure or bearing comprising a plurality of irregular layers or laminations bonded to the base. For the purpose of providing specific corrosion-resisting properties to the base metal when the surface coating of bearing metal would be unsatisfactory for this purpose an intermediate metallic coat may be of value. While a diffusion bond is highly desirable, particularly if it has good physical properties, it is not absolutely necessary.

The thickness of the applied layer metal may vary within relatively wide limits, but for practical purposes thicknesses from about 0.0005 to about 0.050 inch have given satisfactory results. In any particular case, the thickness will be governed by the nature of the material used, its ease of application, its ease of bonding by heat-treatment, and the like. We have produced satisfactory coatings varying from 0.0005 to 0.050 inch and we prefer to keep the coating as thin as possible in order to combine the inherent properties of both base and layer metals. After heat-treat-

ment, the surface of the work may be smooth machined or allowed to remain slightly rough as desired. The thickness of the coating in its final form is in the order of magnitude of about 0.001 inch. When manufacturing the parts to be subsequently treated, they are finished from about 0.0005 inch to about 0.001 inch below the tolerance specified.

The type of finished surface desired is one in which the coating or layer metal has been machined down until minute areas of the base metal starts showing through the coating. In other words, a hill and valley structure in which the exposed tops of the hills are base metal and the valleys are filled with anti-friction metal. The coating is dressed down until the area of exposed base metal is equal to about 20% of the total bearing surface. The ratio of the exposed base metal to the silver-cadmium coating that remains is therefore about 1:4. It is important that the finished bearing surfaces show a uniformly spotted or "leopard skin" effect. It is essential that the base metal mountain or hill tops peeping through the valleys filled with layer metal be finely and evenly distributed. The surface thus obtained gives an appearance in macrostructure similar to the microstructure of the well known bearing metals whose surface microstructure consists of islands of single crystals of a relatively harder constituent surrounded by a matrix of a relatively softer constituent, but the islands in the bearings embodying the present invention are formed of a plurality of relatively hard grains forming a load supporting structure (e. g., of a nickel-copper alloy) surrounded by a matrix or ground mass of soft plastic material (e. g., silver-cadmium alloy).

Figs. 1 and 2 show desirable types of bearing surface. The light areas represent the layer of anti-friction metal, in this embodiment constituted of Ag-Cd alloy, and the dark areas depict the tops of the hills or projections on the roughened bearing face of the base or foundation stratum constituted of aluminum-copper-nickel alloy. These figures illustrate the desired spotted or mottled or variegated finished bearing surface.

Fig. 4 is similar to Fig. 3 and illustrates schematically the embodiment of the invention in which an intermediate layer is used to assist in bonding the outer layer of bearing metal to the base or foundation stratum. The intermediate layer, as described hereinbefore and as understood by those skilled in the art, should be capable of forming a diffusion bond between the layer and the base metals, i. e., should be a metal which

- 5 alloys comparatively easily with the base metal and the bearing metal when exposed in intimate contact therewith at heat treating temperatures. Satisfactory results have been obtained, for example, using tin as the bonding metal between a 10 base of aluminum-copper-nickel alloy and a layer of silver-cadmium bearing metal. Tin has also been used satisfactorily between the same type of 15 base metal and bearing metal layers of silver and phosphor bronze. (See Table I, below.) The 20 application or deposition of a plurality of layers of different metals to the roughened face of the base or foundation stratum produces, prior to the machining or dressing operation, an intermixed or agglomerate body having a plurality of irregular 25 laminations or strata which become bonded to the base during the heat treating step. When the bearing surface is then dressed or machined by any suitable mechanical operations to reduce the bearing to required dimensions and to provide 30 the required smooth surface finish, these irregular strata are cut or cross sectioned at various angles depending upon the angle of slope of the adjacent projection or hill to the surface. The finished surface thus comprises contiguous areas of 35 different metal constituents of the bearing, producing a mottled or variegated bearing surface.

In Table I are summarized the results obtained in a long series of tests on an aluminum-copper-nickel alloy or a copper-nickel alloy which was 40 surfaced with different alloys and was treated in accordance with the principles of the present invention to produce a novel product. In these tests a  $\frac{5}{8}$ " diameter rod was rotated in a 2 inch cubic block of the same metal, without lubrication 45 of any kind and under considerable pressures:

Table I

| Metal for 2 in. cubic block and for $\frac{5}{8}$ " diameter rod | Layer or coating on $\frac{5}{8}$ " diameter rod   | Bonding or diffusion heat treatment (in hydrogen atmosphere) | Load                                                                                | R.P.M. | Time to produce galling                                                      |
|------------------------------------------------------------------|----------------------------------------------------|--------------------------------------------------------------|-------------------------------------------------------------------------------------|--------|------------------------------------------------------------------------------|
| <i>A</i><br>Cu-Ni alloy                                          | None                                               | None                                                         | <i>Pounds</i><br>600-650<br>1,000-2,000<br>2,000<br>2,000<br>2,000                  | 24     | 0.75 to 1.2.                                                                 |
|                                                                  | do                                                 | do                                                           |                                                                                     | 24     | 1.25 to 6.08.                                                                |
|                                                                  | Zinc                                               | do                                                           |                                                                                     | 19     | 23.0 to 35.5.                                                                |
|                                                                  | Chromium plated                                    | do                                                           |                                                                                     | 19     | 3.0.                                                                         |
|                                                                  | Tin                                                | do                                                           |                                                                                     | 19     | 14.0.                                                                        |
|                                                                  |                                                    |                                                              |                                                                                     |        | <i>Minutes</i>                                                               |
| <i>B</i><br>Al-Cu-Ni alloy                                       | None                                               | do                                                           | 1,000-2,000<br>2,000<br>6 hrs. at 420° F.<br>6 hrs. at 420° F.<br>6 hrs. at 420° F. | 20     | 0.20 to 1.66.                                                                |
|                                                                  | Phosphor bronze                                    | do                                                           |                                                                                     | 19     | 8.75-45.0.                                                                   |
|                                                                  | Tin                                                | 6 hrs. at 420° F.                                            |                                                                                     | 19     | 60.0 (surface not galled but slightly sealed).                               |
|                                                                  | Tin and phosphor bronze                            | 6 hrs. at 420° F.                                            |                                                                                     | 19     | 60.0 (surface not galled but slightly sealed).                               |
|                                                                  | Silver and tin                                     | 6 hrs. at 420° F.                                            |                                                                                     | 19     | 60.0 (surface not galled and only slightly sealed).                          |
|                                                                  | Silver and cadmium with tin as intermediate layer. | 2 hrs. at 600° F. followed by 3 hrs at 1000° F.              |                                                                                     | 2,000  | 60.0 (no galling but considerable scaling).                                  |
| Do                                                               | Silver and cadmium                                 | 6 hrs. at 420° F.                                            | 2,000                                                                               | 19     | 60.0 (surface not galled and almost as good at end of test as at beginning). |
|                                                                  | Silver and cadmium                                 | 10 hrs. at 750° F.                                           |                                                                                     | 20     | 60.0 (no galling but some scaling).                                          |

*A* designates a copper-nickel alloy.

*B* designates an aluminum-copper-nickel alloy.

Fig. 3 shows a desirable type of bearing surface in cross section. The polycrystalline "mountains" or "hills" constituted of base metal are peeping through valleys filled with a coating constituted of the anti-friction metal.

These tests show conclusively that the novel product made by the present invention possesses remarkable bearing properties.

A second series of wear or galling tests was conducted on thrust bushings in a traversing gear

box in comparison with a standard bronze bushing, under conditions where the aluminum-copper-nickel alloy could not be used without surface treatment. Table II summarizes the results of this series of tests:

cordance with the principles of the present invention has been in daily continuous service without any of the difficulties previously encountered.

An example showing the excellent resistance to corrosion of the novel product embodying our

Table II

| Type of base metal      | Layer metal                 | Thrust load | Lubrication | Cycles elapsed in test at rate of 85 per min. until first indication of galling occurred | Bonding or diffusion heat treatment  |
|-------------------------|-----------------------------|-------------|-------------|------------------------------------------------------------------------------------------|--------------------------------------|
| Standard bearing bronze | None                        | 1,000       | Castor oil  | 17,054                                                                                   | None                                 |
| Al-Cu-Ni alloy          | Wiped tin                   | 1,000       | do          | 10,750                                                                                   | Do                                   |
| Do                      | Wiped 50-50 lead-tin solder | 1,000       | do          | 4,977                                                                                    | Do                                   |
| Do                      | do                          | 1,000       | do          | 19,283                                                                                   | 3 hrs. in molten solder at 1,040° F. |
| Do                      | do                          | 1,000       | None        | 3,120                                                                                    | Do                                   |
| Do                      | Plated Cd                   | 1,000       | Castor oil  | 16,259                                                                                   | 8 hrs. at 525° F.                    |
| Do                      | Silver solder               | 1,000       | do          | 15,013                                                                                   | 2 hrs. at 1050° F.                   |
| Do                      | do                          | 1,000       | None        | 5,391                                                                                    | Do                                   |

The results of a third series of tests are given in Table III to illustrate the excellent and improved properties of a silver-cadmium surfaced, aluminum-copper-nickel alloy under conditions of sliding and/or rolling friction with heavy pressures and with and without lubrication. The silver-cadmium alloy contained 75-80 per cent of silver and 20-25 per cent of cadmium. For comparative purposes, results are included of one test on an aluminum-copper-nickel alloy, the face of which was not treated according to the present invention.

invention will now be given. An aluminum-copper-nickel alloy had a bonded 75 per cent silver-25 per cent cadmium surface and was exposed 25 continuously in a 4 per cent common salt (NaCl) solution for two weeks. At the end of this period no evidences of corrosion were detected.

Although the present invention has been described in connection with preferred embodiments, it is to be understood that various modifications may be made without departing from the spirit and scope of the invention as described herein and as defined in the appended claims.

Table III

| Example number | Thickness and finish of coating                         | Area tested | Pressure load                         | Type of friction at 140 two inch strokes per min. | Lubrication       | Description                                                                                                                                                                                                      | Results       |
|----------------|---------------------------------------------------------|-------------|---------------------------------------|---------------------------------------------------|-------------------|------------------------------------------------------------------------------------------------------------------------------------------------------------------------------------------------------------------|---------------|
| 1              | 0.020 in. (machined finish).                            | 2 sq. in.   | 1,250 p. s. i.                        | Sliding                                           | Light machine oil | (a) 15 sec. under friction followed by 120 sec. "rest period" to dissipate temperature.<br>(b) 60 sec. under friction and 20 minute "rest period".<br>(c) 6 cycles of 15 sec. of friction and 45 sec. of "rest". | No failure.   |
| 1              | do                                                      | do          | do                                    | do                                                | do                |                                                                                                                                                                                                                  | Do.           |
| 1              | do                                                      | do          | do                                    | do                                                | do                |                                                                                                                                                                                                                  | Do.           |
| 2              | 0.001-0.002 in. (rough finish).                         | 1 sq. in.   | 1,000 lbs. per inch of roller length. | Rolling                                           | Light machine oil | (a) 142 sec. under friction followed by 80 sec. rest.<br>(b) 13 min. under friction followed by 1 hr. rest.<br>(c) 12 cycles of 15 sec. of friction and 45 sec. of "rest".                                       | Do.           |
| 2              | do                                                      | do          | do                                    | do                                                | do                |                                                                                                                                                                                                                  | Do.           |
| 2              | do                                                      | do          | 1,000 p. s. i.                        | Sliding                                           | do                |                                                                                                                                                                                                                  | Do.           |
| 3              | do                                                      | do          | 1,000 lbs. per inch of roller length. | Rolling                                           | None              | (a) 76 min. of friction                                                                                                                                                                                          | Do.           |
| 3              | do                                                      | do          | 1,000 p. s. i.                        | Sliding                                           | do                | (b) 12 cycles of 15 sec. of friction and 45 sec. of rest.<br>(c) 12 cycles of 15 sec. of friction and 45 sec. rest.                                                                                              | Do.           |
| 3              | do                                                      | do          | 2,000 p. s. i.                        | do                                                | do                |                                                                                                                                                                                                                  | Do.           |
| 4              | No anti-galling coating machined Al-Cu-Ni alloy surface | do          | 1,000 p. s. i.                        | Sliding                                           | Light machine oil | (c) 6 sec. of friction                                                                                                                                                                                           | Badly galled. |

p. s. i. indicates pounds per square inch.

A fourth illustrative embodiment of the present invention will now be described. A steel spline shaft, which worked as a machine element under very close tolerances and under considerable pressure, exhibited tendencies to gall and seize in spite of lubrication. The face of this steel spline shaft was provided with a thin 75-25 silver-cadmium alloy layer by electrodeposition. The results have been very satisfactory and successful and the steel spline shaft treated in ac-

70 Thus, small amounts of other elements may be included in the silver-cadmium alloy to favorably influence certain of its properties, e. g., indium to improve corrosion resistance, and copper or nickel up to about 2% to improve the physical properties. In the foregoing description and the following claims the term "bearing face" is applied to the surface or surfaces of the base metal which is or are treated in accordance with the principles of the present invention to form a

"bearing surface," the latter term designating the actual anti-friction and anti-galling surface of the bearing.

We claim:

1. A composite metallic anti-friction and anti-galling bearing comprising a body of copper-nickel alloy and a layer of silver-cadmium alloy bonded together at their interface, the bearing face of the body having a plurality of small approximately equally spaced hills, separated by shallow valleys, over substantially its entire surface, the bearing surface comprising tops of said hills surrounded by a matrix of the cadmium-silver alloy.

2. A composite metallic anti-friction and anti-galling bearing comprising a body of base metal of desired strength but deficient in anti-friction and anti-galling properties and a layer of cadmium-silver alloy containing about 10 to 95% silver and the balance substantially cadmium, the face of said body in contact with said layer being provided with a plurality of small metal hills extending through said layer to provide a bearing surface comprising areas of said metal hills surrounded by a matrix of the cadmium-silver alloy.

3. A composite metallic bearing comprising a body of base metal having a bearing face, and a layer of silver alloy containing about 5 to 35% cadmium anchored to said face by projections from said body extending through said layer.

4. A corrosion resistant bearing comprising a body of nickel alloy possessing strength and corrosion resistance, a plurality of projections on one face of said body, and an adherent layer of bearing metal softer than said nickel alloy body bonded to said face, the bearing surface comprising tops of said projections surrounded by said bearing metal.

5. A bearing adapted for use in contact with sea water, brines and the like comprising a body of nickel-copper alloy possessing strength and corrosion resistance and an adherent layer of silver-cadmium alloy intimately bonded thereto, said body of nickel-copper alloy having a plurality of projections of small cross sectional size extending through the layer of silver-cadmium alloy and forming a minor part of the bearing surface.

6. A composite metallic anti-friction and anti-galling bearing having a bearing surface comprising a plurality of separate irregular macroscopic islands of an alloy comprised largely of nickel and copper constituting a load supporting structure surrounded by a matrix of bearing metal, said islands of nickel-copper alloy forming a minor portion of said bearing surface and said

matrix of bearing metal forming a major portion of said bearing surface.

7. A composite metallic anti-friction and anti-galling bearing having a bearing surface comprising a plurality of separate irregular macroscopic islands of a copper-containing alloy constituting a load supporting structure surrounded by a matrix of bearing metal containing lead, said islands of copper-containing alloy forming a minor portion of said bearing surface and said matrix of lead-containing bearing metal forming a major portion of said bearing surface.

8. A composite metallic anti-friction and anti-galling bearing having a bearing surface comprising a plurality of small separate irregular islands of an alloy comprised largely of nickel and copper constituting a load supporting structure surrounded by a matrix of an alloy comprised largely of lead and tin, said islands of nickel-copper alloy forming a minor portion of said bearing surface and said matrix of lead-tin alloy forming a major portion of said bearing surface.

9. A bearing having a composite surface comprised in major part of a silver-cadmium alloy containing silver as the major constituent and the balance of said surface being small, polycrystalline islands of material harder than the surrounding silver-cadmium alloy.

10. A bearing having a composite surface comprised in part of bearing metal and the balance of said surface being small, polycrystalline islands of nickel alloy harder than the surrounding bearing metal.

11. A composite metallic bearing comprising a body of base metal having a bearing face and a layer of silver alloy containing up to about 2% of at least one metal of the group consisting of nickel and copper anchored to said face by projections from said body extending through said layer.

12. A composite metallic bearing comprising a body of base metal having a bearing face and a layer of an alloy including silver in predominant amounts and the balance substantially cadmium, anchored to said face by projections from said body extending through said layer.

13. A composite metallic bearing comprising a body of base metal having a bearing face and a layer of an alloy comprising about 10% to 95% silver, small amounts of indium effective to increase the corrosion-resistance of the alloy, and the balance substantially cadmium, anchored to said face by projections from said body extending through said layer.

PAUL ETIENNE QUENEAU.  
WILLIAM ALVIN MUDGE.